

1

2,928,789

## MINERAL OIL COMPOSITIONS

Thoburn P. Sands, Maplewood, Mo., assignor to Monsanto Chemical Company, St. Louis, Mo., a corporation of Delaware

No Drawing. Application May 7, 1954  
Serial No. 428,389

14 Claims. (Cl. 252—33.4)

This invention relates to improvements in mineral oil lubricating compositions.

Many oil-soluble additives have been proposed for the purpose of imparting detergent-dispersant properties and oxidation inhibiting properties to mineral oil fractions employed as lubricating oils. In that no one substance satisfactorily imparts both oxidation inhibiting and detergent-dispersant properties to a mineral oil lubricating fraction various combinations of oil-soluble additives have been proposed and while some combinations are satisfactory the art has constantly sought improvements particularly with respect to the more efficient and more economical use of such additives.

Among the more effective additives imparting detergent-dispersant properties to mineral oil lubricating fractions are the oil-soluble metallo hydrocarbon sulfonates, particularly the oil-soluble metallo wax-alkylated aryl sulfonates. However, these detergents tend to increase the oxidation rate of the oil during use and their presence results in an increased concentration of acidic oxidation products in the oil. The increase in the amounts of these acidic oxidation products presents a serious corrosion problem particularly in internal combustion engines which employ alloy bearings. Antioxidants or oxidation inhibiting agents have been added to mineral oil lubricating compositions to prevent or inhibit the formation of mineral oil oxidation products and among the antioxidants proposed for use with the metallo hydrocarbon sulfonate detergent-dispersants are the expensive oil-soluble sulfurized- and phosphorized-dicyclic terpenes. However, while the latter type mineral oil antioxidant and the aforementioned metallo hydrocarbon sulfonate detergent-dispersant separately perform their individual functions in lubricating oils in a highly satisfactory manner, when they are employed in conjunction with one another, particularly over any extended period of time, the full benefit of their individual properties is not realized.

In accordance with this invention it has been found that the detergent-dispersant and oxidation characteristics of a mineral oil fraction of lubricating viscosity containing a minor proportion of a mixture of an oil-soluble phosphorized- and sulfurized-dicyclic terpene antioxidant and an oil-soluble metallo hydrocarbon sulfonate detergent-dispersant is materially improved by incorporating therein a small amount of an oil-soluble sulfurized-monocyclic terpene. Furthermore a more stable and more economical mineral oil lubricating composition is obtained by the incorporation in a mineral oil containing a detergent-dispersant and an antioxidant of the aforesaid types a small amount of a sulfurized-monocyclic terpene.

The amount of oil-soluble sulfurized-monocyclic terpene added to a mineral oil fraction containing an oil-soluble phosphorized- and sulfurized-dicyclic terpene antioxidant and an oil-soluble metallo hydrocarbon sulfonate detergent-dispersant in order to provide a more stable, more efficient and more economical lubricating composition will vary depending upon the circumstances, such as

for example the character of the mineral oil fraction, the concentrations and type of phosphorized- and sulfurized-dicyclic terpene antioxidant and metallo hydrocarbon sulfonate detergent-dispersant, the proposed use of the lubricating composition, and the like. In general the concentrations by weight with respect to the oil base will be 0.1–10% of the metallo hydrocarbon sulfonate detergent-dispersant, 0.05–3% of the phosphorized- and sulfurized-dicyclic terpene antioxidant and 0.05–2% of the sulfurized-monocyclic terpene, however, concentrations of the order of 0.4–5% by weight of the sulfonate detergent-dispersant, 0.1–1% of the phosphorized- and sulfurized-dicyclic terpene, and 0.1–0.5% of the sulfurized-monocyclic terpene with respect to the mineral oil fraction provide a highly efficient and economical lubricating oil composition which is satisfactory for most purposes. A particularly effective and economical lubricating composition is one containing predominantly a mineral oil fraction of lubricating viscosity and with respect to the oil base 0.2–0.4% by weight of an oil-soluble sulfurized-monocyclic terpene, 0.2–0.4% by weight of an oil-soluble phosphorized- and sulfurized-dicyclic terpene, and 0.6–1.2% of an oil-soluble di-wax alkylated benzene sulfonate of an alkaline earth metal such as magnesium, calcium, strontium, or barium. For purposes of this invention magnesium is included in the alkaline earth metal group.

In general a given quantity of a sulfurized monocyclic terpene of this invention upon its incorporation in a lubricating oil composition containing a phosphorized- and sulfurized-dicyclic terpene antioxidant and a metallo hydrocarbon sulfonate detergent-dispersant in effect is equivalent to the incorporation in the oil of approximately an equal weight of a phosphorized- and sulfurized-dicyclic terpene antioxidant and from approximately an equal weight to as much as four to five times its weight of a metallo hydrocarbon sulfonate dispersant-detergent. For example a mineral oil containing 1 part sulfurized-monocyclic terpene, 1.5 parts sulfurized- and phosphorized-dicyclic terpene, and 3 parts metallo hydrocarbon sulfonate is substantially equivalent to a mineral oil containing 2.5 parts of the phosphorized- and sulfurized-dicyclic terpene and 8 parts of the metallo hydrocarbon sulfonate. Thus it is clear by the incorporation of a sulfurized-monocyclic terpene smaller quantities of both the phosphorized- and sulfurized-dicyclic terpene antioxidant and the metallo hydrocarbon sulfonate detergent-dispersant are necessary to provide a highly satisfactory and relatively inexpensive lubricating oil. To give a specific example the following lubricating mineral oil compositions were prepared and evaluated by the Coordinating Research Council L-4-545 and L-1-545 tests and found to exhibit substantially the same oxidation stability and detergent-dispersant properties.

|    | Lubricant Composition                                                                      | Parts by weight |       |
|----|--------------------------------------------------------------------------------------------|-----------------|-------|
|    |                                                                                            | A               | B     |
| 60 | Mineral Oil of Lubricating Viscosity                                                       | 88.25           | 88.75 |
|    | Basic Barium Salt of a Di-wax-alkylated Benzene Sulfonic Acid (16.1% Barium; 3.87% Sulfur) | 1.63            | 0.65  |
|    | Phosphorized- and Sulfurized-Pinene (7.7% Phosphorus, 21.3% Sulfur)                        | 0.52            | 0.31  |
|    | Sulfurized-Dipentene (35% Sulfur)                                                          |                 | 0.22  |

65 By replacing the basic barium salt of the diwax-alkylated benzene sulfonic acid in the above example with the corresponding basic magnesium salt substantially the same results are obtained.

70 As further illustrative of this invention the following lubricating compositions were prepared and evaluated in a CRC Designation L-4-545 (described on page 394

of the CRC Handbook 1946) engine test for oxidation stability:

| Lubricant Composition                                                                      | C               | D               |
|--------------------------------------------------------------------------------------------|-----------------|-----------------|
|                                                                                            | Parts by weight | Parts by weight |
| Mineral Oil of Lubricating Viscosity                                                       | 98.18           | 98.52           |
| Basic Barium Salt of a Di-wax-alkylated Benzene Sulfonic Acid (16.1% Barium; 3.87% Sulfur) | 1.19            | 0.89            |
| Phosphorized- and Sulfurized-Pinene (7.7% Phosphorus, 21.3% Sulfur)                        | 0.63            | 0.27            |
| Sulfurized-Dipentene (35% Sulfur)                                                          |                 | 0.32            |

Table I

|                                                           | Lubricant C | Lubricant D |
|-----------------------------------------------------------|-------------|-------------|
| Bearing Corrosion (mgs. weight loss in metal per bearing) | 81          | 69          |
| Piston varnish rating (based on 10)                       | 8.9         | 9.1         |
| Overall engine rating (based on 100)                      | 86.6        | 88.0        |

As still further illustrative of this invention the following lubricating compositions were prepared and evaluated in a CRC Designation L-1-545 (described on page 347 of the CRC Handbook 1946) engine test for detergent-dispersant properties.

| Lubricating Composition                                                                    | E               | F               |
|--------------------------------------------------------------------------------------------|-----------------|-----------------|
|                                                                                            | Parts by weight | Parts by weight |
| Mineral Oil of Lubricating Viscosity                                                       | 98.66           | 98.61           |
| Basic Barium Salt of a Di-wax-alkylated Benzene Sulfonic Acid (16.1% Barium; 3.87% Sulfur) | 0.84            | 0.82            |
| Phosphorized- and Sulfurized-Pinene (7.7% Phosphorus, 21.3% Sulfur)                        | 0.50            | 0.44            |
| Sulfurized-Dipentene (35% Sulfur)                                                          |                 | 0.13            |

Table II

|                         | Lubricant E                                                               | Lubricant F                                                             |
|-------------------------|---------------------------------------------------------------------------|-------------------------------------------------------------------------|
| Time of Test            |                                                                           |                                                                         |
| No. 1 Groove (top ring) | 240 hours<br>Moderate to heavy<br>hard packed<br>carbon deposit.          | 480 hours.<br>Moderate carbon<br>deposit.                               |
| No. 2 Groove            | Moderate to heavy<br>dark lacquer<br>deposit plus some<br>carbon deposit. | Very light lacquer<br>deposit over<br>half of groove,<br>balance clean. |
| No. 3 Groove            | Moderate to heavy<br>dark lacquer<br>deposit over most<br>of groove.      | Stain on one half<br>of groove,<br>balance clean.                       |
| No. 4 Groove            | Light to moderate<br>dark lacquer<br>deposit over most<br>of groove.      | Clean.                                                                  |
| Piston Skirt            | Trace of amber<br>lacquer deposit<br>on front side.                       | Do.                                                                     |

The oil-soluble sulfurized-monocyclic terpene hydrocarbons of this invention may be prepared by any of the well known methods for sulfurizing unsaturated hydrocarbons such as the direct heating of elemental sulfur with an olefin under pressure. While dipentene is the preferred monocyclic terpene hydrocarbon of this invention other unsaturated monocyclic terpenes of the class described as menthenes and mentadienes, such as for example terpinolene, commercial mixtures of dipentene and terpinolene, limonene, sylvestrene, carvestrene and the like are also suitable. The preferred sulfurized-monocyclic terpene additives are the sulfurized-dipentenes containing 30-40% sulfur by weight, however, any sulfurized-monocyclic terpene containing about 24-50% sulfur by weight is satisfactory. Sulfurized-monocyclic terpenes containing as little as 15% sulfur by weight are also contemplated.

The oil-soluble sulfurized- and phosphorized-dicyclic terpene hydrocarbon antioxidants of this invention are those obtained by reacting a dicyclic terpene hydrocarbon

such as pinene, camphene, fenchene and similar terpenes possessing one double bond in the molecule and comprising two ring systems, with a phosphorus sulfide at a reaction temperature of about 100°-160° C. While any phosphorus sulfide such as  $P_3S_5$ ,  $P_4S_6$ ,  $P_4S_3$ ,  $P_2S_5$ ,  $P_4S_7$ , and the like, may be employed in the preparation of said reaction products, the preferred reaction products are those obtained employing phosphorus pentasulfide. While the proportions of these reactants will vary depending upon the oil-soluble and oil-improvement properties desired the preferred product is that obtained by the reaction of approximately one molecular proportion of a phosphorus sulfide, such as  $P_2S_5$ , with approximately four molecular proportions of a dicyclic terpene, such as pinene, at a reaction temperature of 100°-160° C.

The preferred oil-soluble metallo hydrocarbon sulfonate detergent-dispersants of this invention are those obtained by sulfonating wax-alkylated aromatic hydrocarbons and forming neutral or basic metal salts thereof. 20 This class may be represented by the general formula



where  $n$  is a whole number from 1 to 4, preferably 2, where R is an aromatic hydrocarbon radical such as 25 phenyl, tolyl, xylyl, cumyl, naphthyl, biphenyl, etc. where M is a bivalent metal such as zinc, the alkaline earth metals such as magnesium, calcium, strontium, barium, and the like, where X is  $-SO_3-R-(wax)_n$  or preferably a hydroxyl group. The "wax" substituent or substituents of the preferred detergent-dispersant of this invention consists of carbon and hydrocarbon as distinguished from ester waxes. The hydrocarbon wax substituent contains at least 18 carbon atoms in the lowest carbon chain and is derived from hydrocarbon waxes having 30 melting points varying between about 90° F. and about 180° F. The preferred wax substituents are those known in the art as paraffin waxes which contain at least 20 carbon atoms and usually not more than 30 and which have melting points varying from 90° to 140° F. Other hydrocarbon wax substituents are the cerese waxes which have melting points as high as 180° F. and are derived from petroleum. Other oil-soluble metallo alkylated aryl sulfonate detergent-dispersants are also contemplated for example, those aryl sulfonates containing alkyl groups possessing not less than eight carbon atoms. Other typical oil-soluble hydrocarbon sulfonate detergent-dispersants are those obtained by sulfonating paraffins, naphthenes the various paraffinic, naphthenic and aromatic petroleum fractions and the like, and forming the neutral metal or basic metal salts thereof. 45 As exemplary of the preferred detergent-dispersants are the basic magnesium, neutral magnesium, basic calcium, neutral calcium, strontium, basic barium, and neutral barium salts of di-wax-alkylated benzene sulfonic acids. Other detergent-dispersants within the scope of this invention are the basic barium salt of a diwax-alkylated naphthalene sulfonic acid, the zinc salt of a diwax-alkylated benzene sulfonic acid, the barium salt of a petroleum oil sulfonate.

50 While the invention has been described with respect to certain preferred embodiments it is not so limited in that various modifications may be made which are obvious to those skilled in the art as for example the inclusion of stabilization agents, pour point depressants, extreme pressure lubrication improving agents, viscosity improving agents, and the like, without departing from the spirit or scope of the invention.

This application is a continuation-in-part of co-pending application Serial No. 208,054, filed January 26, 1951, now abandoned.

55 What is claimed is:

1. A lubricating composition comprising a mineral oil and with respect to the mineral oil about 0.1-10% by weight of an oil-soluble metallo hydrocarbon sulfonate detergent, about 0.05-3% by weight of an oil-soluble

phosphorized- and sulfurized-dicyclic terpene, and about 0.05-2% by weight of an oil-soluble sulfurized-monocyclic terpene.

2. A lubricating composition comprising a mineral oil fraction of lubricating viscosity and with respect to the mineral oil fraction about 0.1-10% by weight of an oil-soluble metallo wax-alkylated aromatic hydrocarbon sulfonate detergent, about 0.05-3% by weight of an oil-soluble phosphorized- and sulfurized-dicyclic terpene obtained by reacting a phosphorus sulfide with a dicyclic terpene, and about 0.05-2% by weight of an oil-soluble sulfurized-monocyclic terpene containing 24-50% sulfur by weight.

3. A lubricating composition comprising predominantly a mineral oil fraction of lubricating viscosity and with respect to the mineral oil fraction about 0.1-10% by weight of an oil-soluble basic barium wax-alkylated aryl sulfonate detergent of the general formula



where  $n$  is a whole number from 1-3 inclusive and where  $\text{R}$  is a benzenoid hydrocarbon radical containing but one uncondensed benzene nucleus, about 0.05-3% by weight of a phosphorized- and sulfurized-dicyclic terpene obtained by reacting a phosphorus sulfide with a dicyclic terpene at about 100°-160° C., and about 0.05-2% by weight of a sulfurized-monocyclic terpene containing 30-40% by weight sulfur.

4. A lubricating composition comprising predominantly a mineral oil fraction of lubricating viscosity and with respect to the mineral oil fraction about 0.1-10% by weight of an oil-soluble metallo wax-alkylated aryl sulfonate detergent of the general formula



where  $n$  is a whole number from 1-4, where  $\text{R}$  is an aromatic hydrocarbon radical, where  $\text{M}$  is a divalent metal, and where  $\text{X}$  is selected from the group consisting of a hydroxyl group and  $(\text{wax})_n\text{R}-\text{SO}_3$ , about 0.05-3% by weight of a phosphorized- and sulfurized-dicyclic terpene obtained by reacting about one molecular proportion of a phosphorus sulfide with about four molecular proportions of a dicyclic terpene at about 100°-160° C., and about 0.05-2% by weight of a sulfurized-monocyclic terpene containing 30-40% by weight sulfur.

5. A lubricating composition comprising predominantly a mineral oil fraction of lubricating viscosity and with respect to the mineral oil fraction about 0.1-10% by weight of an oil-soluble metallo wax-alkylated aryl sulfonate detergent of the general formula



where  $\text{M}$  is an alkaline earth metal, about 0.05-3% by weight of a phosphorized- and sulfurized-pinene obtained by reacting substantially one molecular proportion of phosphorus pentasulfide with substantially four molecular proportions of pinene at 100°-160° C., and about 0.05-2% by weight of a sulfurized-dipentene containing 30-40% by weight sulfur.

6. A lubricating composition comprising predominantly a mineral oil fraction of lubricating viscosity and with respect to the mineral oil fraction about 0.1-10% by weight of an oil-soluble metallo wax-alkylated aryl sulfonate detergent of the general formula



where  $\text{M}$  is an alkaline earth metal, about 0.05-3% by

weight of a phosphorized- and sulfurized-pinene obtained by reacting substantially one molecular proportion of phosphorus pentasulfide with substantially four molecular proportions of pinene at 100°-160° C., and about 0.05-2% by weight of a sulfurized-dipentene containing 30-40% by weight sulfur.

7. A lubricating composition comprising predominantly a mineral oil fraction of lubricating viscosity and with respect to the mineral oil fraction about 0.4-5% by weight of an oil-soluble metallo wax-alkylated aryl sulfonate detergent of the general formula



where  $\text{M}$  is an alkaline earth metal, about 0.1-1% by weight of a phosphorized- and sulfurized-pinene obtained by reacting substantially one molecular proportion of phosphorus pentasulfide with substantially four molecular proportions of pinene at 100°-160° C., and about 0.1-0.5% by weight of a sulfurized-dipentene containing 30-40% by weight sulfur.

8. A lubricating composition comprising predominantly a mineral oil fraction of lubricating viscosity and with respect to the mineral oil fraction about 0.4-5% by weight of an oil-soluble metallo wax-alkylated aryl sulfonate detergent of the general formula



where  $\text{M}$  is an alkaline earth metal, about 0.1-1% by weight of a phosphorized- and sulfurized-pinene obtained by reacting substantially one molecular proportion of phosphorus pentasulfide with substantially four molecular proportions of pinene at 100°-160° C., and about 0.1-0.5% by weight of a sulfurized-dipentene containing 30-40% by weight sulfur.

9. A lubricating composition comprising predominantly a mineral oil fraction of lubricating viscosity and with respect to the mineral oil fraction about 0.6-1.2% by weight of an oil-soluble metallo wax-alkylated aryl sulfonate detergent of the general formula



where  $\text{M}$  is an alkaline earth metal, about 0.2-0.4% by weight of a phosphorized- and sulfurized-pinene obtained by reacting substantially one molecular proportion of phosphorus pentasulfide with substantially four molecular proportions of pinene at 100°-160° C., and about 0.2-0.4% by weight of a sulfurized-dipentene containing about 35% by weight sulfur.

10. A lubricating composition comprising predominantly a mineral oil fraction of lubricating viscosity and with respect to the mineral oil fraction about 0.6-1.2% by weight of an oil-soluble metallo wax-alkylated aryl sulfonate detergent of the general formula



where  $\text{M}$  is an alkaline earth metal, about 0.2-0.4% by weight of a phosphorized- and sulfurized-pinene obtained by reacting substantially one molecular proportion of phosphorus pentasulfide with substantially four molecu-

lar proportions of pinene at 100°-160° C., and about 0.2-0.4% by weight of a sulfurized-dipentene containing about 35% by weight sulfur.

11. A lubricating composition comprising predominantly a mineral oil fraction of lubricating viscosity and with respect to the mineral oil fraction about 0.6-1.2% by weight of an oil-soluble barium wax-alkylated aryl sulfonate of the general formula



about 0.2-0.4% by weight of a phosphorized- and sulfurized-pinene obtained by reacting substantially one molecular proportion of phosphorus pentasulfide with substantially four molecular proportions of pinene at 100°-160° C., and about 0.2-0.4% by weight of a sulfurized-dipentene containing about 35% by weight sulfur.

12. A lubricating composition comprising predominantly a mineral oil fraction of lubricating viscosity and with respect to the mineral oil fraction about 0.6-1.2% by weight of an oil-soluble barium wax-alkylated aryl sulfonate of the general formula



about 0.2-0.4% by weight of a phosphorized- and sulfurized-pinene obtained by reacting substantially one molecular proportion of phosphorus pentasulfide with substantially four molecular proportions of pinene at 100°-160° C., and about 0.2-0.4% by weight of a sulfurized-dipentene containing about 35% by weight sulfur.

13. A lubricating composition comprising predominantly a mineral oil fraction of lubricating viscosity and with respect to the mineral oil fraction about 0.6-1.2% 40

by weight of an oil-soluble magnesium wax-alkylated aryl sulfonate of the general formula



about 0.2-0.4% by weight of a phosphorized- and sulfurized-pinene obtained by reacting substantially one molecular proportion of phosphorus pentasulfide with substantially four molecular proportions of pinene at 100°-160° C., and about 0.2-0.4% by weight of a sulfurized-dipentene containing about 35% by weight sulfur.

14. A lubricating composition comprising predominantly a mineral oil fraction of lubricating viscosity and with respect to the mineral oil fraction about 0.6-1.2% by weight of an oil-soluble barium wax-alkylated aryl sulfonate of the general formula



25 where the wax substituent is derived from a paraffin wax containing 20-30 carbon atoms having a melting point of 90-140° F., about 0.2-0.4% by weight of a phosphorized- and sulfurized-pinene obtained by reacting substantially one molecular proportion of phosphorus pentasulfide with substantially four molecular proportions of pinene at 100°-160° C., and about 0.2-0.4% by weight of a sulfurized-dipentene containing about 35% by weight sulfur.

#### References Cited in the file of this patent

#### UNITED STATES PATENTS

|           |         |               |
|-----------|---------|---------------|
| 2,417,305 | Knowles | Mar. 11, 1947 |
| 2,493,216 | Berger  | Jan. 3, 1950  |
| 2,643,248 | Brennan | June 23, 1953 |
| 2,721,862 | Brennan | Oct. 25, 1955 |